

# UNITED STATES PATENT OFFICE.

L. BRANDEIS, OF NEW YORK, N. Y.

## IMPROVEMENT IN PROCESSES OF MAKING BRONZE-POWDERS.

Specification forming part of Letters Patent No. 8,365, dated September 13, 1851.

*To all whom it may concern:*

Be it known that I, LEOPOLD BRANDEIS, in the city of New York, State of New York, have invented a new and Improved Mode of Producing Bronze-Powders, by hand, water, steam, or any other power, and giving the same a handsome, bright appearance; and I do hereby declare that the following is a full and exact description thereof.

The nature of my invention consists in producing the powder by rolling it between steel or iron tempered rollers, instead of the old producing (kept secret) to beat the metal to Dutch leaf and grinding it, to give it a bright and brilliant surface by covering the bronze with soap instead of grease and oil, and polishing the surface by application of polished rollers.

To enable others skilled in the art to make use of my invention, I will proceed and describe its construction and operation, also the old proceeding.

The making of bronze-colors has been carried on in two places in Germany for the last one hundred and fifty years, and is still kept a secret there. As Fürth and Nuremberg, in Bavaria, are the only places in the world where metal-beating is carried on to any great extent, and the waste of the leaf is used for making bronze, they supplied the whole known world. Their expensive process is as follows: After the metal has been reduced by water-power to a ribbon of a thinness of one-sixth of an inch it is beat with iron hammers of twenty-two pounds each till about one-twelfth of an inch thick, annealed, cut in square pieces of one and a half inch, laid between parchment, and beat two hours. Then it is taken out, annealed after wrapping it up in a stout piece of rolled brass, cooled between sand, cleaned, and cut

again in square inch pieces. Then it is filled in the gold-beaters' skins and beat until reduced to the thin leaf, commonly called "Dutch" or "metal" leaf. The cuttings and waste leaf are used now for grinding, after it was brushed through a sieve. Then it is washed out, moved slowly and equally for an hour to settle the metallic parts on the bottom of a basin containing six pounds, then dried. For giving it brilliancy and to protect it against the influence of air, they cover it with grease over a coal-fire. Some even grind it with oil and take the superfluous oil out again by hydraulic pressure.

My proceeding is: I take ship-metal (sheeting) or any other rolled copper or composition of copper, zinc, and tin, break this down by iron or steel rollers to a powder, mix this with gum-arabic and water, grind it an hour, wash it out, and dry it. After this I take half an ounce of white Windsor or any other white soap, scrape it under the bronze, pass the mixture through metallic rollers to polish the bronze, and give it a coat of soap, brush it through a hair sieve to get it clean of small pieces of soap, &c.

What I claim as my invention is—

1. Making metallic bronze-powder of copper, tin, spelter, or their alloys by running them through iron or steel rollers, substantially as described.
2. The application and manner of application of soap to make the bronze bright and brilliant and durable.

L. BRANDEIS.

Witnesses:

L. WICKERT,  
D. NEWMANN.